



US008649704B2

(12) **United States Patent**  
**Gilmartin et al.**

(10) **Patent No.:** **US 8,649,704 B2**  
(45) **Date of Patent:** **Feb. 11, 2014**

(54) **BIAS CHARGING OVERCOAT**

(75) Inventors: **Brian P. Gilmartin**, Williamsville, NY (US); **Liang-Bih Lin**, Rochester, NY (US); **Jeanne M. Koval**, Marion, NY (US); **Aaron M. Stuckey**, Fairport, NY (US); **Gary A. Batt**, Fairport, NY (US)

(73) Assignee: **Xerox Corporation**, Norwalk, CT (US)

(\*) Notice: Subject to any disclaimer, the term of this patent is extended or adjusted under 35 U.S.C. 154(b) by 607 days.

(21) Appl. No.: **12/622,684**

(22) Filed: **Nov. 20, 2009**

(65) **Prior Publication Data**

US 2011/0123220 A1 May 26, 2011

(51) **Int. Cl.**  
**G03G 15/00** (2006.01)

(52) **U.S. Cl.**  
USPC ..... **399/109**; 399/174; 399/176; 492/49; 492/53; 492/56

(58) **Field of Classification Search**  
USPC ..... 399/109, 174  
See application file for complete search history.

(56) **References Cited**

## U.S. PATENT DOCUMENTS

|               |         |                             |
|---------------|---------|-----------------------------|
| 4,899,689 A   | 2/1990  | Takeda et al.               |
| 4,966,675 A   | 10/1990 | Steininger                  |
| 5,017,965 A   | 5/1991  | Hashimoto et al.            |
| 5,068,063 A   | 11/1991 | Tremper, III                |
| 5,678,140 A * | 10/1997 | Fuei et al. .... 399/109    |
| 5,702,812 A * | 12/1997 | Bracken et al. .... 428/323 |
| 5,804,309 A   | 9/1998  | Itoh et al.                 |
| 5,822,169 A   | 10/1998 | Yoshioka et al.             |
| 6,203,855 B1  | 3/2001  | Tarnawskyj et al.           |

|                   |         |                                 |
|-------------------|---------|---------------------------------|
| 6,376,594 B1      | 4/2002  | Sasagawa et al.                 |
| 6,458,883 B1      | 10/2002 | Takashima et al.                |
| 6,728,502 B2 *    | 4/2004  | Hara ..... 399/176              |
| 6,807,389 B2      | 10/2004 | Facci et al.                    |
| 6,889,023 B2 *    | 5/2005  | Suda et al. .... 399/176        |
| 6,915,095 B2      | 7/2005  | Longhenry et al.                |
| 6,962,746 B2      | 11/2005 | Taniguchi et al.                |
| 8,465,893 B2 *    | 6/2013  | Grabowski et al. .... 430/69    |
| 8,483,591 B2 *    | 7/2013  | Lin et al. .... 399/109         |
| 2003/0113650 A1 * | 6/2003  | Suwabe et al. .... 430/120      |
| 2003/0175045 A1 * | 9/2003  | Hara ..... 399/176              |
| 2004/0057749 A1 * | 3/2004  | Saito et al. .... 399/109       |
| 2006/0034636 A1   | 2/2006  | Kosuge et al.                   |
| 2007/0224404 A1   | 9/2007  | Finley et al.                   |
| 2007/0230975 A1   | 10/2007 | Yamazaki et al.                 |
| 2007/0271792 A1   | 11/2007 | Kagawa et al.                   |
| 2008/0232853 A1 * | 9/2008  | Law ..... 399/176               |
| 2009/0180806 A1   | 7/2009  | Oshima et al.                   |
| 2011/0045305 A1 * | 2/2011  | Gilmartin et al. .... 428/423.1 |
| 2011/0207872 A1 * | 8/2011  | Schinkel et al. .... 524/495    |

(Continued)

## FOREIGN PATENT DOCUMENTS

|    |              |        |
|----|--------------|--------|
| EP | 0606907 A1   | 7/1994 |
| JP | 2006163059 A | 6/2006 |

## OTHER PUBLICATIONS

U.S. Appl. No. 12/548,522, Office Action dated Oct. 20, 2011.  
U.S. Appl. No. 12/548,522, Office Action dated Apr. 26, 2012.

(Continued)

*Primary Examiner* — David Gray  
*Assistant Examiner* — Geoffrey Evans

(74) *Attorney, Agent, or Firm* — Hoffman Warnick LLC

(57) **ABSTRACT**

Provide herein is a bias charging member that includes a conductive core, and an outer surface layer disposed on the conductive core. The outer surface layer includes carbon black and polycarbonate.

**10 Claims, 2 Drawing Sheets**



(56)

**References Cited**

**U.S. PATENT DOCUMENTS**

2012/0301818 A1 \* 11/2012 Gilmartin et al. .... 430/66  
2013/0004205 A1 \* 1/2013 Gilmartin et al. .... 399/176  
2013/0236721 A1 \* 9/2013 Law, Kock-Yee .... 428/339

**OTHER PUBLICATIONS**

Wenderoth, U.S. Appl. No. 12/622,682, Office Action, Apr. 17, 2013,  
32 pages.

Wenderoth, U.S. Appl. No. 12/548,522, Notice of Allowance & Fees  
Due, Mar. 13, 2013, 9 pages.

Wenderoth: U.S. Appl. No. 12/548,522, Office Action Nov. 26, 2012,  
19pgs.

Wenderoth, U.S. Appl. No. 12/622,682, Office Action Communica-  
tion, Aug. 22, 2013, 21 pages.

Wenderoth, U.S. Appl. No. 12/622,682, Office Action Communica-  
tion, Dec. 13, 2013.

\* cited by examiner



FIG. 1



**FIG. 2**



**FIG. 3**

## 1

## BIAS CHARGING OVERCOAT

## TECHNICAL FIELD

The disclosure herein relates to overcoat layers, and more specifically, to an outer surface layer of carbon black and polycarbonate for xerographic members such as bias charging members.

## BACKGROUND

In a conventional charging step included in electrophotographic processes using an electrophotographic photosensitive member, in most cases a high voltage (DC voltage of about 5-8 KV) is applied to a metal wire to generate a corona, which is used for the charging. In this method, however, a corona discharge product such as ozone and  $\text{NO}_x$  is generated along with the generation of the corona. Such a corona discharge product deteriorates the photosensitive member surface and may cause deterioration of image quality such as image blurring or fading or the presence of black streaks across the copy sheets. Further, ozone contamination may be harmful to humans if released in relatively large quantities. In addition, a photosensitive member that contains an organic photoconductive material is susceptible to deterioration by the corona products.

Also, as the power source, the current directed toward the photosensitive member is only about 5 to 30% thereof. Most of the power flows to the shielding plate. Thus, the efficiency of the charging means is low.

For overcoming or minimizing such drawbacks, methods of charging have been developed using a direct charging member for charging the photosensitive member. For example, U.S. Pat. No. 5,017,965 to Hashimoto et al., uses a charging member having a surface layer which comprises a polyurethane resin. Another approach, European Patent Application 0 606 907 A1, uses a charging roller having an elastic layer comprising epichlorohydrin rubber, and a surface layer thereover comprising a fluorine containing bridged copolymer.

These and other known charging members are used for contact charging a charge-receiving member (photoconductive member) through steps of applying a voltage to the charging member and disposing the charging member being in contact with the charge-receiving member. Such bias charging members require a resistivity of the outer layer within a desired range. Specifically, materials with resistivities which are too low will cause shorting and/or unacceptably high current flow to the photoconductor. Materials with too high resistivities will require unacceptably high voltages. Other problems which can result if the resistivity is not within the required range include nonconformance at the contact nip, poor toner releasing properties and generation of contaminant during charging. These adverse affects can also result in bias charging members having non-uniform resistivity across the length of the contact member. It is usually the situation that most of the charge is associated at or near the center of the charge member. The charge seems to decrease at points farther away from the center of the charge member. Other problems include resistivity that is susceptible to changes in temperature, relative humidity, running time, and leaching out of contamination to photoconductors.

Due to its contact, the direct charging apparatus also causes more wear and tear to itself, imaging members and any other components with which it comes in contact. Failure modes in a bias charge roller (BCR) show up in prints such as dark streaks, and white and dark spots, which are associated with

## 2

surface damages on BCR. These defects are usually derived from degradation or debris build-up on the BCR surface along the circumference, i.e. the process direction. The degradations can be scratches, abrasion, or pothole-like damages to the BCR surface. Another known deficiency is toner filming on the BCR surface that can also show up as print streaks. All these failures will reduce BCR life and therefore limit usage life.

10

## SUMMARY

There is described a bias charging member that includes a conductive core, and an outer surface layer disposed on the conductive core. The outer surface layer includes a conductive additive and polycarbonate.

There is further described a method of refurbishing a bias charging member. The method includes obtaining a bias charging member having a conductive core and an outer surface. A dispersion of a carbon black and polycarbonate is coated on the outer surface. The coating is heated to form a conductive overcoat.

There is further described a bias charging member that includes a conductive core and an outer surface layer on the conductive core. The surface layer includes carbon black and a polymer, wherein the outer surface layer has a surface resistivity of equal to or greater than about  $1 \times 10^{13}$  ohm/, an average modulus of from about 3.50 to about 5.00 GPa and an average hardness of from about 250 to about 500 MP.

30

## BRIEF DESCRIPTION OF THE DRAWINGS

FIG. 1 demonstrates an illustrative bias charging roll (BCR) having an electrically conductive core and an outer surface layer provided thereon.

FIG. 2 shows a scanned image print output from a BCR having an outer surface layer in accordance with an aspect herein.

FIG. 3 shows a scanned image print output from a standard BCR.

## DETAILED DESCRIPTION

Referring to FIG. 1, there is shown an embodiment having a bias charging roller (BCR) 2 held in contact with an image carrier implemented as a photoconductive member 3. However, embodiments herein can be used for charging a dielectric receiver or other suitable member to be charged. The photoconductive member 3 may be a drum, a belt, a film, a drelt (a cross between a belt and a drum) or other known photoconductive member. While the BCR 2 is in rotation, a DC voltage and optional AC current is applied from a power source 9 to a electro-conductive core 4 of the BCR 2 to cause it to charge the photosensitive member 3. Shown in FIG. 1, the electro-conductive core 4 is surrounded by a base material 5. Although shown as one layer, it is possible to eliminate the base material 5 or have multiple layers of base material 5. These layers are referred to as base layers, intermediate layers or substrate layers. The base material 5 for the BCR 2 can be any elastic material with semiconductive dopant of suitable fillers discussed below. A semiconductive protective overcoat is provided on the base material 5 of the BCR 2 to form the outer surface layer 7. There may or may not be a filler in the substrate layer, intermediate layer, and outer layer.

The protective overcoat layer or outer surface layer 7 contains semiconductive carbon black in polycarbonate. The density of the carbon black was about  $264 \text{ kg/m}^3$ .

The electro-conductive core **4** serves as an electrode and a supporting member of the charging roll, and is composed of an electro-conductive material such as a metal or alloy of aluminum, copper alloy, stainless steel or the like; iron coated with chromium or nickel plating; an electro-conductive resin and the like. The diameter of the electro-conductive core is, for example, about 1 mm to about 20 cm, or from about 5 mm to about 2 cm.

The base materials can be isoprene rubber, chloroprene rubber, epichlorohydrin rubber, butyl rubber, polyurethane, silicone rubber, fluorine rubber, styrene-butadiene rubber, butadiene rubber, nitrile rubber, ethylene propylene rubber, epichlorohydrin-ethylene oxide copolymer rubber, epichlorohydrin-ethylene oxide-allyl glycidyl ether copolymer rubber, ethylene-propylene-diene terpolymer copolymer rubber (EPDM), acrylonitrile-butadiene copolymer rubber (NBR), natural rubber, and blends thereof. Among these, polyurethane, silicone rubber, EPDM, epichlorohydrin-ethylene oxide copolymer rubber, epichlorohydrin-ethylene oxide-allyl glycidyl ether copolymer rubber, NBR, and blends thereof are preferably used.

An electro-conductive agent, an electronic electro-conductive agent or an ionic electro-conductive agent may be used in the base material **5**. Examples of the electronic electro-conductive agent include fine powder of: carbon black such as Ketjen Black and acetylene black; pyrolytic carbon, graphite; various kinds of electro-conductive metal or metal alloy such as aluminum, copper, nickel and stainless steel; various kinds of electro-conductive metal oxide such as tin oxide, indium oxide, titanium oxide, tin oxide-antimony oxide solid solution, and tin oxide-indium oxide solid solution; insulating materials having a surface treated by an electro-conductive process; and the like. Furthermore, examples of the ionic electro-conductive agent include perchlorates or chlorates of tetraethylammonium, lauryltrimethyl ammonium and the like; perchlorates or chlorates of alkali metal such as lithium and magnesium, and alkali earth metal; and the like. These electro-conductive agents may be used alone, or in combination of two or more kinds thereof.

Furthermore, the amount of addition to the base material **5** is not particularly limited. For example, the amount of the electronic electro-conductive agent to be added is from about 1 to about 30 parts by weight, or from about 5 to about 25 parts by weight with respect to 100 parts by weight of the rubber material. The amount of the ionic electro-conductive agent to be added is in the range of about 0.1 to about 5.0 parts by weight, or from about 0.5 to about 3.0 parts by weight with respect to 100 parts by weight of the rubber material. The layer thickness of the base material is from about 10 mm to about 20 cm, or from about 50 mm to about 3 cm.

The protective overcoat layer is composed of polycarbonate and a conductive agent such as carbon black. The carbon black loading is directly correlated to the surface resistivity of the material. The amount of the electro-conductive agent to be added is not particularly limited. For example, the amount of electro-conductive agent can be in the range of about 0.1 to about 40 by weight, or from about 4 to about 9 parts by weight, or in the range of about 6 to 7 parts by weight with respect to 100 parts by weight of the total weight of the coating. The layer thickness of the protective overcoat layer is from about 0.1  $\mu$ m to about 500  $\mu$ m, or from about 1  $\mu$ m to about 50  $\mu$ m.

The structure of the polycarbonate in the outer surface layer **7** may include but is not limited to derivatives of bisphenol A polycarbonate (PCA), bisphenol C polycarbonate (PCC), bisphenol F polycarbonate (PCF), bisphenol Z polycarbonate (PCZ) and the like. The polycarbonate has a weight

average molecular weight ( $M_w$ ) in the range from about 100,000 to about 500,000. The outer surface layer has an average modulus of from about 3.50 to about 5.00 GPa and an average hardness of from about 250 to about 500 MPa. Surprisingly, a higher resistivity is possible using polycarbonate, a material that possesses a high surface hardness, than with softer materials.

There may be present a conductive filler in any one of the substrate layers, intermediate layers or overcoat layers. Conductive fillers include those listed previously as electro-conductive agents and particles and carbon fillers such as carbon black, graphite, fluorinated carbon, and the like; conductive polymer fillers such as polyaniline, polypyrrole, polythiophene, polyacetylene and the like; metal fillers such as silver, copper, antimony and the like; metal oxide fillers such as titanium oxides, zinc oxides antimony tin oxides and the like

There may be present non-conductive fillers in the substrate layers or intermediate layers.

The protective overcoat **7** also allows for refurbishing of the BCR **2**. By applying a protective overcoat **7** to a BCR **2** having a damaged surface, either the base material **5** or the outer surface, a BCR can be used multiple times. When the outer surface of the BCR **2** becomes too damaged to provide acceptable prints, it is returned for refurbishing. Refurbishing involves applying a protective overcoat **7** as described herein. After application of the surface layer, the BCR is typically heated to remove any residual solvent.

Since BCRs usually can last in machine for many thousand cycles, accelerated testing was performed with a print cartridge wear test fixture. The protocol for the testing involves initial screening (time=0), which involves resistance and charge uniformity measurements, and print test. The BCR was subjected to wear for 50,000 cycles in the wear fixture, followed by a screening under the same procedures as the time=0 screening. The same process continued, i.e. screening at successive 50 thousand intervals in the wear fixture, until significant print streaks appeared.

## EXAMPLE 1

The overcoat dispersion was prepared by ball milling a sample of PCZ 400, a polycarbonate available from Mitsubishi Gas Chemical Co., with 5 wt % Vulcan XC72 carbon black (Cabot) in THF. The sample was ball milled for 3 days, after which the dispersion was filtered. The resistivity of the material was measured to be  $10^{13} \Omega/\square$ . The sample was then coated on a BCR using a Tsukiage coater giving a 6  $\mu$ m overcoat. The BCR was then dried in a convection oven at 135° C. for 15 min to remove any solvent.

Charge uniformity measurements of the BCR with polycarbonate/carbon black overcoat and regular BCRs with no overcoat at time equal zero and after 50,000 cycles were compared. The charge uniformity of overcoated BCRs was comparable to the standard BCR without any overcoats before and after the wear test, suggesting there is no internal electric build-up in the overcoat layers and no deterioration in the charging capability with the addition of the overcoat.

Start and running torques of the overcoated BCRs were comparable with standard BCRs and the results are consistent with print and wear test, as no noticeable torque issues were detected.

Print testing of the BCR with the polycarbonate overcoat showed significant improvement over prints obtained from the BCR with no overcoat. FIG. 2 shows a print image from a Pinehurst machine equipped with the polycarbonate overcoated BCR after 50,000 cycles wear on the Hodaka fixture.

## 5

No print defects were observed from this BCR after subjecting it to 50 kcycle wear. In contrast, FIG. 3 shows the print obtained from the control BCR with no overcoat, in which significant streaking is observed.

In summary, an overcoat for a BCR composed of a polycarbonate polymer doped with carbon black significantly improves print quality compared to a BCR with no overcoat. The overcoated BCR displays excellent charge uniformity, which is comparable to a BCR with no overcoat. After subjecting the overcoated BCR to 50,000 cycles wear on a Hodaka fixture, no black streaks were observed, which is in contrast to prints obtained from a BCR with no overcoat as shown in FIG. 3.

It will be appreciated that a variety of the above-disclosed and other features and functions, or alternatives thereof, may be desirably combined into many other different systems or applications. Various presently unforeseen or unanticipated alternatives, modifications, variations, or improvements therein may be subsequently made by those skilled in the art, which are also intended to be encompassed by the following claims.

We claim:

**1. A bias charging member comprising:**

- a) a conductive core,
- b) a base material selected from the group consisting of isoprene rubber, chloroprene rubber, epichlorohydrin rubber, butyl rubber, polyurethane, silicone rubber, fluorine rubber, styrene-butadiene rubber, butadiene rubber, nitrile rubber, ethylene propylene rubber, epichlorohydrin-ethylene oxide copolymer rubber, epichlorohydrin-ethylene oxide-allyl glycidyl ether copolymer rubber, ethylene-propylene-diene terpolymer copolymer rubber, acrylonitrile-butadiene copolymer rubber (NBR) and natural rubber disposed on the conductive core, wherein the base material has a thickness of from about 10 mm to about 20 cm; and

an outer surface layer disposed on the base material, the outer surface layer comprising a conductive additive and polycarbonate wherein the outer surface layer has a surface resistivity of equal to or greater than about  $1 \times 10^{13}$  ohm/and wherein the outer surface layer has a thickness of from about 0.1  $\mu\text{m}$  to about 500  $\mu\text{m}$ .

**2. The bias charging member in accordance with claim 1, wherein the conductive additive comprises carbon black in an amount from about 0.1 to about 40 percent by weight based on a weight of total solids in the outer surface layer.**

**3. The bias charging member in accordance with claim 1, wherein the conductive additive comprises carbon black in an amount from about 4 to about 9 percent by weight based on a weight of total solids in the outer surface layer.**

**4. The bias charging member in accordance with claim 1, wherein the outer surface layer comprises an average modulus of from about 3.50 to about 5.00 GPa.**

**5. The bias charging member in accordance with claim 1, wherein the outer surface comprises an average hardness of from about 250 to about 500 MPa.**

**6. A method of refurbishing a bias charging member comprising:**

## 6

obtaining a bias charging member having a conductive core, a base material selected from the group consisting of isoprene rubber, chloroprene rubber, epichlorohydrin rubber, butyl rubber, polyurethane, silicone rubber, fluorine rubber, styrene-butadiene rubber, butadiene rubber, nitrile rubber, ethylene propylene rubber, epichlorohydrin-ethylene oxide copolymer rubber, epichlorohydrin-ethylene oxide-allyl glycidyl ether copolymer rubber, ethylene-propylene-diene terpolymer copolymer rubber, acrylonitrile-butadiene copolymer rubber (NBR) and natural rubber, the base material disposed on the conductive core, wherein the base material has a thickness of from about 10 mm to about 20 cm, and an outer surface;

coating a dispersion of a carbon black and polycarbonate on the outer surface; and

heating the coating to form a conductive overcoat wherein the conductive overcoat has a surface resistivity of equal to or greater than about  $1 \times 10^{13}$  ohm/and wherein the conductive overcoat has a thickness of from about 0.1  $\mu\text{m}$  to about 500  $\mu\text{m}$ .

**7. The method of claim 6, wherein the conductive overcoat has an average modulus of from about 3.50 to about 5.00 GPa.**

**8. A bias charging member comprising:**

- a) a conductive core,
- b) a base material selected from the group consisting of isoprene rubber, chloroprene rubber, epichlorohydrin rubber, butyl rubber, polyurethane, silicone rubber, fluorine rubber, styrene-butadiene rubber, butadiene rubber, nitrile rubber, ethylene propylene rubber, epichlorohydrin-ethylene oxide copolymer rubber, epichlorohydrin-ethylene oxide-allyl glycidyl ether copolymer rubber, ethylene-propylene-diene terpolymer copolymer rubber, acrylonitrile-butadiene copolymer rubber (NBR) and natural rubber disposed on the conductive core, wherein the base material has a thickness of from about 10 mm to about 20 cm; and

an outer surface layer provided on the base material and comprising a carbon black and polycarbonate, wherein the outer surface layer has a surface resistivity of equal to or greater than about  $1 \times 10^{13}$  ohm/, an average modulus of from about 3.50 to about 5.00 GPa, an average hardness of from about 250 to about 500 MP and a thickness of from about 1  $\mu\text{m}$  to about 50  $\mu\text{m}$ .

**9. The bias charging member in accordance with claim 8, wherein carbon black comprises an amount from about 0.1 to about 40 percent by weight based on a weight of total solids in the outer surface layer.**

**10. The bias charging member in accordance with claim 8, wherein carbon black comprises an amount from about 4 to about 9 percent by weight based on a weight of total solids in the outer surface layer.**

\* \* \* \* \*